

Sept. 12, 1972

H. YAMAGISHI ET AL  
PREVENTING RUSTING OF STEEL SHEETS COATED WITH  
AQUEOUS SLURRY OF METAL POWDER  
Filed Nov. 17, 1970

3,690,940



## 1

3,690,940

### PREVENTING RUSTING OF STEEL SHEETS COATED WITH AQUEOUS SLURRY OF METAL POWDER

Hidehisa Yamagishi, Fumitoshi Yokoi, and Tadao Takahashi, Kawasaki, Japan, assignors to Nippon Kokan Kabushiki Kaisha

Filed Nov. 17, 1970, Ser. No. 90,379

Claims priority, application Japan, Nov. 21, 1969,  
44/93,141

Int. Cl. B22f 7/04; C23c 17/00

U.S. Cl. 117—131

2 Claims

#### ABSTRACT OF THE DISCLOSURE

In coating steel sheet with aqueous slurry of metal powder, the slurry is added with corrosion inhibitor to prevent rusting of steel sheet at the time of drying the coating layer thereby improving the adhesion thereof to the steel surface, said corrosion inhibitor addition being a compound containing any one of such negative ions as  $\text{NO}_2^-$ ,  $\text{MoO}_4^{2-}$  or  $\text{C}_6\text{H}_5\text{COO}^-$  in a concentration ranging from  $10^{-5}$  mol/l. to  $10^{-1}$  mol/l.

The present invention relates to a metal coating method for steel sheets, and more particularly to a method of improving on the adhesion of metal coating layer to the surface of the steel sheet by restraining rusting of the steel sheet which is coated with metal powder in accordance with the water-slurry method at the stage of drying said metal coating layer.

As for the method of coating surface of steel sheets with a slurry which is prepared by admixing metal powder and a solution, there are one or two methods known in the prior art. However, there is yet no established technique relating to the use of corrosion inhibitor as an additive to suppress the rusting of steel sheet. Therefore, the adhesion of coating layers and steel sheets is always reduced in any of the conventional methods as the steel surface starts rusting at the stage of drying subsequent to coating. And it has been the common practice to use organic solvents in lieu of water in order to obviate such drawbacks. This is still defective in that it may very well lead to generation of poisonous gas and danger of fire as well as it is expensive, although the use of organic solvent may help restrain the rusting.

Under the afore-mentioned circumstances, the present invention has been developed to provide a novel and useful method in improving on the adhesion of a metal coating layer by modifying the conventional water-slurry coating method in adding a corrosion inhibitor instead of organic solvent so as to prevent rusting of steel sheet. More particularly, it comprises coating steel sheet with a slurry of metal powder, drying, rolling and heat-treating the same. Said slurry contains one or more of the compounds which contain any one of such negative ions as  $\text{NO}_2^-$ ,  $\text{MoO}_4^{2-}$ ,  $\text{C}_6\text{H}_5\text{COO}^-$  in a concentration ranging from  $10^{-5}$  mol/l. to  $10^{-1}$  mol/l.

Reference is now made to the accompanying drawing in which the curves show the effect of the corrosion inhibitors employed in the present invention. Very small amount of said corrosion inhibitors is added to the water-slurry of metal powder in coating the same on steel sheet. As the curves indicate, the amount to be added may vary in accordance with the types of inhibitors used, but is within the range of from  $10^{-5}$  mol/l. to  $10^{-1}$  mol/l. It is desirable that the corrosion inhibitor is a compound containing any one of such negative ions as  $\text{NO}_2^-$ ,  $\text{MoO}_4^{2-}$ , and  $\text{C}_6\text{H}_5\text{COO}^-$ , which is soluble in water and which would not chemically react with the particles of metal powder.

## 2

As is evidently understood from the drawing, the concentration of the inhibitor to be added is specified as in the range from  $10^{-5}$  mol/l. to  $10^{-1}$  mol/l. because:

- 5 (1) no effect thereof can be expected when said concentration is less than  $10^{-5}$  mol/l., thereby it is determined that  $10^{-5}$  mol/l. is the minimum required amount; on the other hand,  
(2) the addition of the corrosion inhibitor exceeding  $10^{-1}$  mol/l. may impair the adhesion of coating layer to steel sheet or the finish of the surface, thereby it is determined that  $10^{-1}$  mol/l. is the upper limit of the range which will not deteriorate the coating layer.

The addition may be carried out by adding any one or more of the corrosion inhibitors into water to dissolve therein, to which metal powder is introduced to prepare a slurry.

Application of coating is not restricted to any particular method nor means, and can be done in accordance with the generally practiced ways such as curtain-flow method, spray method or methods using bar-coaters, roll-coaters or brushes.

After being coated with a slurry, the steel sheet will be heated to such an extent as to dry the coating layer or 25 to have the metal particles sinter slightly. It is then subjected to rolling in order to improve on the adhesion of the coating layer to the steel sheet. The coating layer after the rolling should show hardening due to the workings, and thus it becomes inferior in the drawability. By removing the warping due to the workings under such heat-treatment conditions as inhibit the formation of alloyed layer between the coating layer and the steel sheet, metal coated steel sheet having excellent adhesion and workability may be obtained.

35 In case drawing is necessary, it is desirable to conduct temper rolling after the heat-treatment.

#### EXAMPLE 1

Slurry containing 1,500 g. of aluminum powder,  $10^{-5}$  mol/l. of  $\text{NaNO}_2$  and 1,000 g. of water is coated on steel sheet with a reverse roll-coater to have the coating layer after drying weigh 80 g./m.<sup>2</sup>. After drying the coating layer, the steel sheet is rolled to elongate by 7%, and then subjected to heat-treatment in an oxidizing atmosphere of 600° C. for 2 minutes.

The resultant product has a gloss surface and is superior in anti-corrosiveness and workability.

#### EXAMPLE 2

50 Slurry containing 1,500 g. of aluminum powder,  $10^{-3}$  mol/l. of  $\text{Na}_2\text{MoO}_4$  and 1,200 g. of water is applied on a steel sheet with the use of a bar-coater.

The amount of coating is 75 g./m.<sup>2</sup> when weighed after 55 drying. The steel sheet thus coated is then subjected to heat-treatment in an oxidizing atmosphere for 30 seconds in a furnace temperature of 650° C. and to rolling to elongate by 5%. It is further treated for post-aging treatment in an electric furnace the temperature of which is maintained at 400° C. and rolled for temper regulation.

60 The resultant product is of the same properties as that of Example 1, and exhibits anti-corrosiveness for more than 1,200 hours when subjected to salt spray test (JIS-Z2371).

#### EXAMPLE 3

65 Slurry containing 1,500 g. of aluminum powder,  $10^{-4}$  mol/l. of  $\text{C}_6\text{H}_5\text{COONa}$ ,  $10^{-5}$  mol/l. of  $\text{Na}_2\text{MoO}_4$  and 1,000 g. of water is applied on steel sheet with the use of sprayer. It is subjected to succeeding procedures identical to those of Example 1 such as drying and rolling. The amount of coating weighed after drying is 75 g./m.<sup>2</sup>. The ratio of elongation at the time of rolling is 5%. The heat-

treatment is conducted in accordance with the induction heating system which is so controlled as to raise the temperature of the steel surface to 500° C., in two minutes.

The resultant product is of the same properties as those of Examples 1 and 2. It is superior in anti-corrosiveness, and peeling-off of the coating layer is not observed when formed into sash (window frame).

As can be understood from the foregoing description, the present invention enables the improvement of the adhesion of coated layer to steel sheet since the rusting or corrosion at the time of drying is suppressed in steel sheet coated with water-soluble paint and water-slurry. The employment of water in lieu of organic solvent as the dispersing agent in the present invention is economically advantageous. The present invention eliminates danger of fire as compared with the conventional method, as well as it is harmless to bodies. Thus, numerous advantages can be expected of the present invention. Also, it may well be applicable to all the corrosion preventive methods in the field wherein a coating is formed on steel sheet with the use of water as a medium such using water-soluble paint, water-slurry, water-soluble emulsion or the like.

What is claimed is:

1. In the method of applying a metal coating layer on a steel sheet wherein a steel sheet is contacted with a slurry of a metal powder and water following by drying, rolling to improve adhesion of the coating layer to the steel sheet and heat-treating to improve workability thereof, the improvement which comprises so contacting said steel sheet with an aqueous slurry of metal powder containing a water-soluble compound containing an ion selected from the group consisting of  $\text{NO}_2^-$ ,  $\text{MoO}_4^{2-}$  and

$\text{C}_6\text{H}_5\text{COO}^-$ , in a concentration of from about  $10^{-5}$  mol/l. to about  $10^{-1}$  mol/l.

2. In the method of applying a metal coating layer on a steel sheet wherein a steel sheet is contacted with a slurry of a metal powder and water following by drying, rolling and heat-treating, the improvement which comprises so contacting said steel sheet with an aqueous slurry of metal powder containing an ion selected from the group consisting of  $\text{NO}_2^-$ ,  $\text{MoO}_4^{2-}$  and  $\text{C}_6\text{H}_5\text{COO}^-$ , in a concentration of from about  $10^{-5}$  mol/l. to about  $10^{-1}$  mol/l.

#### References Cited

#### UNITED STATES PATENTS

|    |           |         |                  |             |
|----|-----------|---------|------------------|-------------|
| 15 | 2,927,043 | 3/1960  | Stetson          | 117—131 X   |
|    | 3,041,206 | 6/1962  | Long et al.      | 117—131     |
|    | 3,231,971 | 2/1966  | McFarland et al. | 117—131 X   |
|    | 3,310,870 | 3/1967  | Parikh et al.    | 29—420.5    |
|    | 3,316,625 | 5/1967  | Flint et al.     | 29—420.5    |
| 20 | 3,395,027 | 7/1968  | Klotz            | 117—131 X   |
|    | 3,432,334 | 3/1969  | Yenawine et al.  | 117—131 X   |
|    | 3,453,849 | 7/1969  | Clarke et al.    | 29—420.5 X  |
|    | 3,479,258 | 11/1969 | Ashcroft         | 29—420.5 X  |
|    | 3,052,575 | 9/1962  | Crane            | 148—6.14 R  |
| 25 | 3,460,977 | 8/1969  | Golben           | 106—1 X     |
|    | 3,351,504 | 11/1967 | DeHart           | 146—6.14 RX |

ALFRED L. LEAVITT, Primary Examiner

J. R. BATTEN, Jr., Assistant Examiner

U.S. Cl. X.R.

29—420.5; 106—1; 148—6.14 R

UNITED STATES PATENT OFFICE  
CERTIFICATE OF CORRECTION

Patent No. 3,690,940 Dated September 12, 1972  
Inventor(s) H. YAMAGISHI et al

It is certified that error appears in the above-identified patent  
and that said Letters Patent are hereby corrected as shown below:

Column 4 - Claim 2 should be rewritten as follows:

"The method of Claim 1, wherein the metal  
powder is aluminum powder."

Signed and sealed this 16th day of April 1974.

(SEAL)

Attest:

EDWARD M. FLETCHER, JR.  
Attesting Officer

C. MARSHALL DANN  
Commissioner of Patents